

## UNITED STATES PATENT OFFICE

2,160,911

## FLUSHING OIL

Robert P. Russell, Elizabeth, N. J., assignor to  
Standard Oil Development Company, a corpora-  
tion of Delaware

No Drawing. Application September 28, 1934,  
Serial No. 745,937

## 5 Claims. (Cl. 87-9)

This invention deals with the use of superior flushing oils and the manufacture thereof. More specifically, it concerns the production of engine-conditioning flushing oils, and will be more clearly understood from the following description.

The usual flushing oils of commerce are mainly employed to remove dirt and sludge from the engine, so as to prevent contamination of the fresh lubricating oil to be added. They comprise 0 oils having little or no lubricating power, such as kerosenes, gas oils and the like. Heretofore, the sole purpose of the flushing oil has been to remove sludge deposits from the engine and no attempts have been made to use a flushing oil 5 which will condition the engine so as to prepare the hot metal surfaces to resist deterioration of the oil.

It is well known that metals such as iron, nickel, etc., act as oxidation catalysts, thereby 0 causing rapid deterioration of the oil. When this occurs, the engine surfaces become coated with undesirable materials decreasing the efficiency and increasing the wear of the engine. "Engine-conditioning" contemplates an effect on the engine metal surfaces such that the catalytic acceleration of lubricating oil deterioration thereby is inhibited or stopped and possibly such that an opposite effect is produced, in which the metal surfaces become active to inhibit ordinary deterioration in the engine. Engine-conditioning agents, whatever may be their mode of operation, 5 have been found to decrease formation and deposition of oxidation and other carbonaceous oil products, and in keeping such products of deterioration in suspension in the oil or as a flocculated mass in the crankcase, not only increase efficiency of the engine but also its life. The flushing oils prepared according to this invention are made engine-conditioning by the addition 0 of materials such as colloidal lead and other metals, metallic soaps such as lead naphthenate, zinc sulfonate, tin naphthenate, etc., other metal-containing organic compounds, as for example those capable of producing colloidal metals on heat treatment, including metallo-organic compounds such as lead tetra-ethyl, tin tetrphenyl, triphenyl bismuth and oil soluble organo-metallic compounds of mercury, arsenic, antimony, zinc, and other materials of the same nature. 5 The surface treatment of the metals by these conditioning agents is considerably different from the usual electro-plating methods in that, generally, with the conditioning agents, no visible change in the appearance of the treated metal

can be noticed with the naked eye, yet such treatment has a profound effect in reducing the formation of carbon or sludge, reducing wear in the engine and increasing the life of the lubricant used. On the other hand, electro-plated 5 surfaces generally become loosened in a short while, and are not very effective, possibly due to porosity, the type of film obtained, etc.

These engine-conditioning materials may be used in any combination desired, preferably in a 10 concentration of 2 to 5% in the flushing oil base. In many cases 0.01 to 0.1 or 1% has been found satisfactory, while in many instances over 2%, say 5% or even 10% or more have been found desirable, depending on the particular agent used, 15 the type of lubricating oil to be added to the engine, the type of engine, and other factors.

Any flushing oil base is suitable for carrying these engine-conditioning agents, although it is preferable to employ oils of low viscosity such as 20 to 30 or 35 seconds Saybolt at 210° F. and especially oil solvents having a kauri butanol value above 20 and, better yet, above 30 or 40. The materials described in application Serial No. 729,234, filed by G. L. Matheson and R. Rosen 25 on June 6, 1934, have been found very suitable for the purposes herein set forth.

In carrying out this invention, the engine-conditioning agents are dissolved or dispersed in the desired flushing oil base stock. A dispersing 30 and/or stabilizing agent may be advantageously added to prevent settling of these materials. The blend so prepared is then added to the engine, the oil of which has been previously drained, and the engine is allowed to run for 5, 10, 15 or 35 even 30 minutes or longer until the lubricating oil has been substantially replaced by the flushing oil. The latter is then drained out and the lubricating oil to be used is added. The flushing oil can be added hot, say at a temperature of 40 100 to 300° F. or higher in order to shorten the time of flushing. It is also often advantageous to flush the engine first with an ordinary flushing oil so as to remove the greater part suspended 45 sludge and solid particles, and then flush with the flushing oil made according to this invention, to recondition the engine. By this means it is possible to save the drainings of the latter step for further flushing purposes, with or without 50 a preliminary purification by filtration, etc. The usual period of operation between flushings depends on the type of oil, and also the engine, but it is found that the effect produced by the present improved flushing oil persists and ordi-

narily it is possible to safely extend the mileage between oil changes. It is desirable to use the flushing oil between all changes but in many instances the improvement is sufficiently persistent so that the flushing may be employed only after two or three oil changes.

The following examples are submitted to show the variety of phases embraced by this invention:

10 *Example 1*

|                                               | Percent |
|-----------------------------------------------|---------|
| Colloidal lead                                | 0.2     |
| Flushing oil, viscosity 30 to 210° F. Saybolt | 99.8    |

15 *Example 2*

|                                                                                   | Percent |
|-----------------------------------------------------------------------------------|---------|
| Lead tetraethyl                                                                   | 0.2     |
| Alpha naphthol                                                                    | 0.2     |
| Petroleum oil of 20-35 viscosity Saybolt at 210° F. and kauri butanol value of 35 | 99.6    |

20 *Example 3*

|                 | Percent |
|-----------------|---------|
| Tin naphthenate | 1.5     |
| Flushing oil    | 99.5    |

25 This blend is heated to 200° F. before introduction into the engine.

Example 4

|                                                       | Percent |
|-------------------------------------------------------|---------|
| Tetraphenyl tin                                       | 1.0     |
| Edeleanu extract (25-35 viscosity Saybolt at 210° F.) | 99.0    |

30 Two samples of flushing oil containing 0.2% triphenyl bismuth were kept in a steel cone (by stoppering the outlet), one for a period of 3 days, 35 the other for 3 hours, at a temperature of about 200° F., corresponding to maximum crankcase temperature. Subsequently the flushing oil was run out of the cone but no visible change was 40 observed. A sample of a lubricating oil run immediately afterwards on this cone at 250° C. without any cleaning gave a marked reduction in deposit as shown by the data given below:

|    | Oil                                                                                | Total cone deposit |
|----|------------------------------------------------------------------------------------|--------------------|
|    | Lubricating oil before flushing                                                    |                    |
| 50 | Lubricating oil after flushing with triphenyl bismuth as described above (3 hours) | Gms. 0.51          |
|    | Lubricating oil after flushing with triphenyl bismuth as described above (3 days)  | 0.43               |
|    |                                                                                    | 0.14               |

55 The cone test is a laboratory method for indicating the tendency of an oil to deposit carbon and other solid or semi-solid products on metal surfaces, and has been found to correlate satisfactorily with actual engine tests. This test involves the dropping of a definite quantity of oil on a heated metal cone grooved in such a manner 60 as to allow a long time of contact for the oil with the metal.

*Example 5*

A sample of flushing oil containing 0.2% tri-

phenyl bismuth was run over the steel cone for a period of five minutes at 250° C. and then lubricating oil was run on the cone at 250° C. without any cleaning up of the cone surface. In another test, the same flushing oil was run over the cone for a period of 15 minutes at 250° C. and then the lubricating oil run without any cleaning up of cone surface. The results obtained as compared with the data on the lubricating oil run on a clean cone at 250° C. are given below:

|                                                                                                                                               | Total cone deposit | Gms. | 15 |
|-----------------------------------------------------------------------------------------------------------------------------------------------|--------------------|------|----|
| 1 Lubricating oil                                                                                                                             |                    |      |    |
| 2 Flushing oil containing 0.2% triphenyl bismuth was run over cone for 5 minutes at 250° C. and then lubricating oil run without any cleaning |                    | 0.43 |    |
| 3 Same as (2) except that flushing oil was run over cone for period of 15 minutes (instead of 5)                                              |                    | 0.26 |    |

20 These engine-conditioning agents may be used in conjunction with oiliness agents, sludge dispersers, oxidation inhibitors, soaps, pour inhibitors, thickeners capable of raising the viscosity and/or viscosity index of oils, also dyes, organic solvents, etc.

25 Various modifications may be made in carrying out this invention, and it is not intended to limit the scope of the description or examples, but only by the following claims in which it is intended to cover the invention as broadly as the prior art permits.

I claim:

30 1. A flushing oil comprising a petroleum oil of the class consisting of kerosene and gas oil, and 35 0.01 to 10% of a metallo-organic compound capable of reducing the cone deposit of the lubricating oil subsequently employed in the engine.

2. A flushing oil comprising a petroleum oil of the class consisting of kerosene and gas oil and 40 0.01 to 5% of an oil soluble metallo-organic derivative of the elements of the group consisting of lead, bismuth, arsenic, antimony, tin and zinc.

3. A flushing oil comprising a petroleum oil solvent for hydrocarbon oils and their decomposition products, and of the class consisting of kerosene and gas oil in which has been incorporated a minor percentage of an oil soluble metallo-organic derivative of an element of the group consisting of lead, bismuth, arsenic, antimony, tin and zinc. 45

4. A flushing oil comprising a petroleum oil solvent for hydrocarbon oils and their decomposition products, and of the class consisting of kerosene and gas oil, in which has been incorporated a minor percentage of a metallic engine conditioning agent selected from the group consisting of colloidal metals and metallo-organic compounds. 55

5. A flushing oil according to claim 4 in which the metallic engine conditioning agent is colloidal lead. 60

ROBERT P. RUSSELL.